

3,068,060

TREATMENT OF CELLULOSE TEXTILES  
WITH PHOSPHORAMIDES

William D. Emmons, Huntingdon Valley, and William S. Wadsworth, Jr., Elkins Park, Pa., assignors to Rohm &amp; Haas Company, Philadelphia, Pa., a corporation of Delaware

No Drawing. Filed Aug. 3, 1959, Ser. No. 831,065  
12 Claims. (Cl. 8—116.2)

The present invention concerns crease-proofing cellulosic fabrics by the application thereto of compounds of the class of polyamides of phosphoric acid.

The compounds with which the cellulosic fabrics are treated in accordance with the present invention are phosphoroamides having the formula



wherein X is selected from the group consisting of —OR, —NHR<sup>0</sup>, and



in which R is a C<sub>1</sub>—C<sub>4</sub> alkyl group, and R<sup>0</sup> and R' are the same or different C<sub>1</sub>—C<sub>4</sub> alkyl groups. Preferred compounds are those in which R, R', and/or R<sup>0</sup> is or are methyl groups.

Examples of these compounds include:

Methyl phosphorodiamide,  
Ethyl phosphorodiamide,  
n-Propyl phosphorodiamide,  
Isopropyl phosphorodiamide,  
n-Butyl phosphorodiamide,  
Isobutyl phosphorodiamide,  
N-methyl phosphotriamide,  
N,N-dimethyl phosphotriamide,  
N,N-diethyl phosphotriamide, and  
N,N-dibutyl phosphotriamide.

In the utilization of the compounds of Formula I for the modification of cellulosic fabrics for crease-proofing, crush-proofing, reduction of shrinkage and stabilization against dimensional changes on washing, the treated cellulosic fabrics exhibit outstanding durability to washing and dry-cleaning and retain their improvement in crease-resistance and shrinkage-reduction even after washing in the usual detergents which are commonly alkaline in character. The treated cellulosic products are also resistant to ordinary acid souring applied in laundries after the washing and rinsing stages. The cellulosic products obtained by treatment with the new compounds are also insoluble because of their cross-linked character so that the improvements in shrinkage and crease-resistance are obtained even after dry-cleaning operations. The treated fabrics also retain excellent hand and feel.

The treatment of the cellulosic fabrics with the phosphoroamides in accordance with the present invention may be effected most advantageously by means of aqueous solutions, dispersions, or emulsions in which the phosphoroamide is dissolved, dispersed or emulsified at a concentration which may vary from 1 to 30% by weight. Preferably, the concentration is from 5 to 15% to obtain the maximum benefits in crease-proofing and shrinkage reduction. The treatment may be carried out in the presence of a catalyst. As a catalyst there may be used metal salts of acids having the composition H<sub>a</sub>(XY<sub>b</sub>), where H is hydrogen, a is an integer which depends on the valence of the complex ion and may have a value of 1 to 3, X is a non-metal selected from the group consisting of boron, silicon, sulfur, and chlorine, said non-

metal being in a state where its valence is from 3 to 7, Y is fluorine or oxygen, and b is an integer having a value of 4 or 6. The metals of these salts are those of groups Ib, II, IIIb, IV, and VIII of the periodic table in T. Moeller, "Inorganic Chemistry," John Wiley & Sons, New York, 1952, which have an atomic weight of at least 12. Salts of perchloric and fluoboric acids are very efficient catalysts, particularly their zinc, lead, copper, and magnesium compounds. Salts of sulfuric acid, such as aluminum and copper sulfate, and of fluosilicic acid, such as magnesium, zinc, and copper fluosilicates, also are active as catalysts. Other acidic compounds, such as acetic acid, phosphoric acid, and sodium bisulfate, may also be used as catalysts. Other catalysts which are especially useful are ammonium phosphate, ammonium thiocyanate, and mixtures of 1 mole of formaldehyde with 1 mole of the hydrochloric or other acid salts of a hydroxy aliphatic amine including 2-methyl-2-amino-1-propanol, 2-methyl-2-amino-1,3-propanediol, tris(hydroxy)aminomethane, 2-phenyl-2-amino-1-propanol, 2-methyl-2-amino-1-pentanol, 2-aminobutanol, triethanolamine, 2-amino-2-ethyl-1-butanol, also ammonium chloride, pyridine hydrochloride, benzylidimethylamine oxalate. The amine salts are water-soluble latent catalysts substantially neutral at ordinary temperature but dissociate into volatile components one of which is acidic at the elevated temperatures used for baking and curing, so that the catalyst after exerting its accelerating effect is automatically discharged during the heating or curing stage.

Conveniently, the amount of catalyst may vary from about 0.2% to 5% and is preferably in the range of 0.5% to 1% concentration in the aqueous solution of the phosphoroamide.

The catalyzed solution, dispersion, or emulsion of the phosphoroamide is compatible with solutions or dispersions of most of the common textile finishing agents, such as synthetic polymer latices and aminoplast resins or pre-condensates, so that they may be applied with the phosphoroamide to produce changes in the hand or other properties of the fabric.

The aqueous solution, dispersion, or emulsion containing the phosphoroamide and catalyst may be applied to the fabric in any suitable manner such as by spraying or impregnation. In general, it is preferable to use some method of impregnation. With piece goods, this is conveniently carried out with the various machines used for treating fabrics in open width, such as pads or jigs. However, it is not required that the impregnation be carried out in open width, and the fabric may be handled in any form. In treating garments or other articles made from cellulosic fabrics, the impregnation may be carried out in a tumble wheel, laundry machine, or other suitable equipment. After application of the solution, dispersion, or emulsion, it is desirable to remove any excess by squeezing the fabric between rollers, or by shaking or centrifuging it, in order to insure a more even treatment. The treated fabric may then be dried, such as by air-drying at normal room temperature or by heating in a dry-ing oven at temperatures of 140° F. and up. The drying and curing operations are preferably done with the fabric open and flat, so that it will have a smooth and even appearance when finished. In a preferred embodiment, the impregnated fabric, immediately after impregnation and without preliminary low-temperature drying is carried in open width by a tenter frame through a curing oven where it is subjected to temperatures of about 212° F. to about 450° F. or higher for a period of time ranging from about one minute to about one-half hour or more, the shorter period being employed at the higher temperature and vice versa. A "flash" cure at 700° to 750° F. for 1 to 20 seconds may be used. Entirely satisfactory results are obtained by heating for ten minutes at about

300° F. This curing operation not only dries the impregnated fabric but apparently causes a reaction between the phosphoroamide and the hydroxyl groups of the cellulose.

The following examples illustrate the present invention, the parts and percentages therein being by weight unless otherwise noted. The crease-recovery values given below are those determined by the Shirley Institute Procedure (British Standard Notebook No. 11, 1949 Edition, page 128) and are the average of warp and filling values

$$\left( \frac{W+F}{2} \right)$$

*Example 1*

(a) A piece of 80 x 80 cotton printcloth was saturated with an aqueous solution containing 10% of N,N-dimethyl phosphotriamide and 1.0% of a 1:1 mole ratio mixture of formaldehyde and the hydrochloride of 2-amino-2-methyl-propanol-1. It was dried for five minutes at 220° F. and then heated for five minutes at 340° F. to complete the insolubilization and cross-linking of the cellulosic material in the fabric. After conditioning, the sample had a crease-recovery angle of 110°. The fabric was 25 resistant to wrinkling and showed no discoloration on washing and ironing.

(b) By carrying out the same treatment but with 1.0% of acetic acid as the catalyst and a cure at 315° F. for 15 minutes, a crease-recovery angle of 113° was reached. 30 The fabric was resistant to wrinkling and showed no discoloration on washing and ironing.

*Example 2*

(a) A similar piece of cotton printcloth was saturated with an aqueous solution containing 10% of methyl phosphorodiamide and 1.5% of zinc perchlorate. It was dried for five minutes at 220° F. and then heated for five minutes at 340° F. to complete the insolubilization and cross-linking of the cellulosic material in the fabric. 40 After conditioning, the sample had a crease-recovery angle of 120°. The fabric was resistant to wrinkling and showed no discoloration on washing and ironing.

(b) The crease-resistance of rayon was improved in similar fashion when the process of part (a) was repeated replacing the cotton fabric with regenerated cellulose fabrics of spun rayon and filament rayon yarns. The fabric was resistant to wrinkling and showed no discoloration on washing and ironing.

*Example 3*

Example 2(a) was repeated but with ethyl phosphorodiamide used at a concentration of 10% and with a mixture of 1% of zinc perchlorate and 0.5% of acetic acid used as the catalyst. The recovery angle was 102°. 55 The fabric was resistant to wrinkling and showed no discoloration on washing and ironing.

*Example 4*

An 80 x 80 cotton printcloth was saturated with an aqueous solution containing 10% of isobutyl phosphorodiamide and 1% of acetic acid. After drying, heating, and conditioning as in Example 1, the fabric was resistant to wrinkling and showed no discoloration on washing and ironing.

It is to be understood that changes and variations may be made without departing from the spirit and scope of the invention as defined by the appended claims.

We claim:

1. A process comprising impregnating a cellulose textile with an aqueous medium containing an acid catalyst and 1 to 30% by weight of a phosphoroamide of the formula



wherein X is a member selected from the group consist-

ing of  $—NHR^0$  and



in which R' is a C<sub>1</sub>—C<sub>4</sub> alkyl group, and R<sup>0</sup> is a C<sub>1</sub>—C<sub>4</sub> alkyl group, drying, and heating the impregnated fabric at a temperature of at least about 212° F.

2. A process comprising impregnating a cellulose textile with an aqueous medium containing an acid catalyst and 1 to 30% by weight of N,N-dimethyl phosphotriamide, drying, and heating the impregnated fabric at a temperature of at least about 212° F.

15 3. A process comprising impregnating a cellulose textile with an aqueous medium containing an acid catalyst and 1 to 30% by weight of cellulose-cross-linking material consisting of methyl phosphorodiamide, drying, and heating the impregnated fabric at a temperature of at least about 212° F.

20 4. A process comprising impregnating a cellulose textile with an aqueous medium containing an acid catalyst and 1 to 30% by weight of cellulose-cross-linking material consisting of ethyl phosphorodiamide, drying, and heating the impregnated fabric at a temperature of at least about 212° F.

5. A process comprising impregnating a cellulose textile with an aqueous medium containing an acid catalyst and 1 to 30% by weight of cellulose-cross-linking material consisting of isobutyl phosphorodiamide, drying, and heating the impregnated fabric at a temperature of at least about 212° F.

6. As an article of manufacture, a fabric comprising cellulose fibers modified by reaction with a phosphoro-



35 wherein X is a member selected from the group consisting of  $—NHR^0$  and



in which R' is a C<sub>1</sub>—C<sub>4</sub> alkyl group, and R<sup>0</sup> is a C<sub>1</sub>—C<sub>4</sub> alkyl group, the modification being effected by the process of claim 1.

7. As an article of manufacture, a fabric comprising cellulose fibers modified by reaction with N,N-dimethyl phosphotriamide by the process of claim 2.

8. As an article of manufacture, a fabric comprising cellulose fibers modified by reaction with methyl phosphorodiamide by the process of claim 3.

9. As an article of manufacture, a fabric comprising cellulose fibers modified by reaction with ethyl phosphorodiamide by the process of claim 4.

10. As an article of manufacture, a fabric comprising cellulose fibers modified by reaction with isobutyl phosphorodiamide by the process of claim 5.

11. A process comprising impregnating a cellulose textile with an aqueous medium containing an acid catalyst and 1 to 30% by weight of cellulose-cross-linking material consisting of at least one (C<sub>1</sub>—C<sub>4</sub>)-alkyl phosphorodiamide, drying, and heating the impregnated fabric at a temperature of at least about 121° F.

12. As an article of manufacture, a fabric comprising cellulose fibers modified by reaction with cellulose-cross-linking material consisting of at least one (C<sub>1</sub>—C<sub>4</sub>)-alkyl phosphorodiamide by the process of claim 11.

References Cited in the file of this patent

UNITED STATES PATENTS

2,832,745 Hechenbleikner ----- Apr. 29, 1958  
2,957,018 Baker ----- Oct. 18, 1960